

## UNITED STATES PATENT OFFICE

2,163,753

## METHOD OF MAKING HOT MOLDING DIE PLATES AND OTHER CASTINGS AND PRODUCT THEREOF

Harry K. Ihrig, Milwaukee, Wis., assignor to  
Globe Steel Tubes Co., Milwaukee, Wis., a corporation of DelawareNo Drawing. Application May 25, 1937,  
Serial No. 144,639

9 Claims. (Cl. 22—203)

This invention pertains to cast metal articles comprising a cast body portion having embedded therein a preformed metallic insert, and it is particularly applicable to articles comprising a body portion cast around a metallic tube to provide a tubular passageway in the article.

In various hot molding operations, such as the manufacture of gaskets and the molding of synthetic resins, there are used cast die plates which must be heated, say to 200° to 400° F., as by means of a steam coil passing through the mid-section of the plate. For the most part the coils for these purposes have been provided by drilling the solid cast plate from the edges to provide one or more passageways parallel with the main, or die, surfaces, the holes not needed but unavoidable in such production being then plugged. Such operations are expensive, and in addition the plates are not wholly satisfactory because such drilled passageways necessarily provide sharp corners at the ends which cause substantial resistance to steam flow and accumulation of scale and corrosion products which may, and frequently do, ultimately stop up the passageway or so insulate it that efficient heat transfer is not possible.

Attempts to make such articles by casting the body metal around tubes disposed in a mold have likewise not produced satisfactory results. A major reason for this has been inefficient heat transfer from fluid passed through the tube. For instance, pyrometric measurement of the molding surface of die plates made in this manner has shown that the temperature at the surface may be as much as 30° below that of the heated fluid, such as steam, supplied to the tube. Also, the temperature at different points on the surface of the plate is not uniform. Sectioning of such plates has shown also that blow holes, or voids, always occur in the casting in the vicinity of the surface of the tube, and apparently the presence of these voids throughout the structure is responsible for the poor heat transfer and non-uniformity of temperature at the die surface.

It is among the objects of this invention to provide cast articles having metallic inserts embedded therein which are characterized by a sound structure, ease and simplicity of production, and by the possession of satisfactory physical properties.

A particular object is to provide cast articles provided with passageways for circulation of fluid, such as hot molding dies, which are characterized by efficient heat transfer between the fluid and the surface of the article, by acceptable uniformity of temperature over the surface, and

which are readily producible and avoid disadvantages heretofore encountered in the art.

It is among other objects of the invention to provide a process of making articles of the type referred to which is simple, readily practiced, not expensive, and produces articles in which the insert is satisfactorily bonded to the cast body of the article, and which are structurally sound.

The invention is predicated upon my discovery that its stated objects are attained by the use of preformed metallic inserts, which are capable of alloying with silicon, and which, at least in those portions which are to be embedded in the casting, are provided with a silicon-rich surface coating. I have discovered that when such preformed inserts having a silicon-rich surface coating are disposed in a mold and metal is cast about them, the silicon present at the surface of the insert is at least incipiently fused and effects satisfactory bonding with the cast metal, and that it further acts to produce a sound casting free, or substantially free, from blow holes and the like defects which have been encountered heretofore in attempting to make such articles. In consequence good heat transfer is afforded between a fluid passed through the tube and the surface of the article, and at the same time uniformity of surface temperature is achieved.

The silicon coating may be provided in a variety of ways, but I now prefer to provide it by silicon cementation of the insert to provide a siliconized case, most suitably one that is rich in silicon. A variety of procedures have been proposed for this purpose but I now prefer to effect the silicon cementation in accordance with the process disclosed and claimed in my Patent No. 2,109,485, dated March 1, 1938, reissued May 10, 1938, as Reissue Patent No. 20,719.

In accordance with the invention of my aforesaid application the article to be cemented is heated to a temperature above about 1500° F., desirably to about 1800° F., in a non-oxidizing atmosphere, and after the article is at heat it is contacted with a silicon-impregnating reagent formed by heating a silicon-supplying material, such as silicon, ferrosilicon or silicon carbide, in contact with chlorine gas or a chloride vapor.

In the preferred practice of that invention the article to be cemented is packed in contact with the silicon-supplying material, in finely divided condition, in a closed container in which they are heated to the cementing temperature. When the article has reached that temperature chlorine gas is introduced, whereupon uniform impregnation of the article takes place readily and rapidly.

By controlling the temperature used and the time of exposure, the depth of the silicon impregnation and the concentration of silicon in the surface may be controlled according to need.

5 While the article is being heated the presence of oxidizing conditions should be avoided. This may be done by passing a current of non-oxidizing gas, such as nitrogen, hydrogen, or mixtures thereof, through the container. The same result 10 may be achieved through the use of the solid residue resulting from a previous cementing operation. I have found also that oxidation does not occur to a detrimental extent if the article is packed in, for example, silicon carbide in a 15 container closed except for conduits for introducing chlorine gas and for outflow of effluent gases, whereby the use of inert gas may be dispensed with.

For the purposes of the present invention the 20 depth of impregnation need not be great provided the surface be rich enough in silicon to effect the desired bonding and absence of blow holes in the cast product. With ferrous metals satisfactory depth may be had by packing the article 25 in silicon carbide, heating to about 1850° F., and then passing chlorine through the container for two to three hours. Cases containing about 14 per cent of silicon may be obtained in this manner.

30 The cases thus produced are well bonded to the underlying metal, and when the cast metal is poured into the mold the silicon-rich surface is fused to an extent such as to insure excellent bonding of the cast body and the insert. Also, 35 blow holes and voids do not form in the cast body near the tubes. This may be due to deoxidation by the silicon, but I do not limit myself to that assumption.

These cases are likewise highly resistant to 40 corrosion, and by silicon cementing both the inside and the outside of the tube, advantage may be taken of this property to insure high resistance to corrosion by fluid media passed through the tube. In the production of cemented tubes it is 45 desirable to rotate the tubes during the cementing operation, particularly where both the inside and outside surfaces of the tubes are to be cemented. Rotation during cementation insures the production of cases of uniform thickness at 50 both surfaces of the tubes, but the tubes should not be rotated too rapidly if thick cases are desired on the outside surface. Also, where maximum resistance to corrosion is desired the steel should contain less than about 0.05 per cent of 55 sulfur.

In another embodiment of the invention of my 60 application aforesaid the insert is heated in a container in a non-oxidizing atmosphere to a temperature as stated above, and there is then introduced into the container a reagent gas produced by heating the silicon-supplying material in a current of chlorine or chloride vapor in a 65 separate container. For some purposes this embodiment is less desirable than that just described because where the cementing gas is formed in a separate container it is necessary that the silicon-supplying material be heated to a temperature of at least about 2300° F.

The inserts provided with silicon-rich 70 surfaces in the foregoing of any other suitable manner are disposed in a mold and the metal, such as iron or steel, is then cast about them. The tubes are, of course, disposed in the relation which they are to bear in the finished casting, and they may be arranged to provide nipples 75

extending outwardly from the casting for connection to a source of fluid which is to be flowed through the tubes. If the tubes do not protrude the connections may be made by tapping and threading the openings in the casting, or in 5 other manners known in the art.

As exemplifying the benefits which flow from the present invention, reference may be made to tests of hot molding dies produced in accordance with it. In one test  $\frac{3}{8}$  inch iron pipe size 10 seamless steel tubes, threaded on both ends, were treated in accordance with the process disclosed in my aforesaid application by heating them in an electric rotating furnace with silicon carbide to a temperature of 1815° F. When the pipes 15 reached that temperature chlorine was passed through the furnace for two and one-half hours, producing a case about 0.02 inch thick. Two of these tubes, 12½ inches long, were then supported in a mold productive of a plate 2 inches 20 by 4 inches by 9 inches, with the threaded ends of the tubes disposed to protrude from the casting, and cast iron at about 2700° F. was poured into the molds to produce the castings. Two such castings were connected by couplings threaded 25 to the ends of the tubes, and steam at 360° F. was then introduced into one tube to flow through the tubes of both castings, a steam tray being connected to the exit end. Readings taken with a 30 pyrometer at the plate surface showed a maximum deviation of 3° to 4° F. from the steam temperature, and the temperature over the entire surface was satisfactorily uniform. The castings were then cut open and found to be free 35 from blow holes in the vicinity of the tube surfaces. Microscopic examination of polished sections showed the siliconized case to have been fused with and bonded to the cast iron.

Other plates were made in similar manner using semi-steel as the cast metal, and these 40 plates exhibited the same heat transfer and structural properties.

Although the invention has been described with particular reference to the use of tubular inserts, it will be understood by those skilled in 45 the art that it is equally applicable to the manufacture of castings embodying inserts of other types, such as solid inserts, inserts of irregular shape, inserts extending wholly or partially through the casting, and the like. Also, various 50 modes of forming coils, using tubes, are possible, as by using a plurality of tubes protruding from the casting and which are connected by suitable fittings, or by forming a coil from tubes and fittings and casting metal entirely around it. 55 And while the invention has been described with particular reference to ferrous metals, it will be understood that it is applicable generally to metals capable of cementation or alloying with silicon. 60

According to the provisions of the patent statutes, I have explained the principle and method of construction of my invention and have described what I now consider to represent its best embodiment. However, I desire to have it 65 understood that, within the scope of the appended claims, the invention may be practiced otherwise than as specifically described.

I claim:

1. That method of making a ferrous metal 70 casting provided with a ferrous metal insert, comprising providing a preformed ferrous metal insert member with an integral silicon-rich cemented case, placing said member in a mold in such position as to have said silicon-rich case 75

surrounded by metal cast therein, and casting ferrous metal into the mold, said silicon-rich case effecting bonding between said insert member and said cast metal, and the casting being substantially free from blowholes in the vicinity of said insert member.

2. That method of making a ferrous metal casting provided with a ferrous metal insert, comprising providing a preformed ferrous metal insert member with an integral silicon-rich cemented case at least in those portions which are to lie within the casting, placing said member in a mold in such position as to have said silicon-rich case surrounded by metal cast therein, and casting into the mold to surround said preformed and cased member ferrous metal heated to a temperature above the melting point of said silicon-rich case, said case effecting bonding between said insert member and said cast metal, and the casting being substantially free from blowholes in the vicinity of said insert member.

3. That method of making a ferrous metal casting provided with a tubular passageway therethrough, comprising providing a ferrous metal tube with an integral silicon-rich cemented case on the portions of the tube which are to lie within the casting, disposing the cased tube in a mold so as to have said silicon-rich case surrounded by metal cast therein, and casting molten ferrous metal into the mold at a temperature above the melting point of said silicon-rich case, said silicon-rich case effecting bonding between said tube and said cast metal, the casting being substantially free from blowholes in the vicinity of said tube, and the tube forming a tubular passageway through the casting.

4. A method according to claim 3, said case containing about 14 per cent of silicon.

5. A cast ferrous metal article comprising a cast ferrous metal body portion and a preformed ferrous metal insert embedded in and surrounded by said cast portion and having a silicon-rich surface formed integrally therewith and bonding said cast portion to said insert, and the casting being substantially free from blowholes in the vicinity of said silicon-rich surface.

6. A cast ferrous metal article according to claim 5, said insert being a wrought ferrous metal tube.

7. A cast ferrous metal article comprising a cast body portion and a wrought ferrous metal tube embedded therein and surrounded thereby, said tube having its inner and outer surfaces provided with an integrally formed silicon-rich cemented case which bonds said cast portion to the outer surface of the tube, and the casting being substantially free from blowholes in the vicinity of said outer surface.

8. A hot molding die or the like comprising a cast ferrous metal body portion having at least one wrought ferrous metal tube embedded therein and surrounded thereby, the outer surface of said tube having an integrally formed silicon-rich cemented case bonding the tube to said cast body portion, and the casting being substantially free from blowholes in the vicinity of said outer surface.

9. A cast ferrous metal article comprising a cast body portion and a wrought ferrous metal tube embedded therein and having its outer surface provided integrally with a silicon-rich cemented case containing about 14 per cent of silicon bonding said tube to said cast body portion, and the cast body portion being substantially free from blowholes in the vicinity of said tube.

HARRY K. IHRIG.